

No. 802,153.

PATENTED OCT. 17, 1905.

H. S. BLACKMORE.

PROCESS OF REDUCING METALS AND MAKING ALLOYS.

APPLICATION FILED JAN. 6, 1905.

2 SHEETS—SHEET 1.

Fig. 1.



Fig. 3.



Fig. 4.



Fig. 2.



Investor

Witnesses

Edwin L. Bradford  
H. N. Jenkins

Henry Spence Blackmore,

No. 802,153.

PATENTED OCT. 17, 1905.

H. S. BLACKMORE.  
PROCESS OF REDUCING METALS AND MAKING ALLOYS.

APPLICATION FILED JAN. 6, 1905.

2 SHEETS-SHEET 2.

FIG. 5.



FIG. 6.



FIG. 7.



Inventor

Henry Spenser Blackmore

Witnesses

Edwin L. Bradford

H. N. Jenkins

# UNITED STATES PATENT OFFICE.

HENRY SPENCER BLACKMORE, OF MOUNT VERNON, NEW YORK.

## PROCESS OF REDUCING METALS AND MAKING ALLOYS.

NO. 802,153.

Specification of Letters Patent.

Patented Oct. 17, 1905.

Original application filed August 22, 1904, Serial No. 221,748. Divided and this application filed January 6, 1905. Serial No. 239,935.

To all whom it may concern:

Be it known that I, HENRY SPENCER BLACKMORE, a citizen of the United States, residing at Mount Vernon, in the county of Westchester and State of New York, have invented certain new and useful Improvements in Processes of Reducing Metals and Making Alloys, being a division from Serial No. 221,748, (Patent No. 775,060,) of which the following is a specification.

The object of my invention is to reduce metals from their oxides and produce alloys thereof in a rapid, efficient, and economical manner; and it consists, essentially, in liquefying compound metal oxides or compounds of metal oxide with other metals by the action of molten oxides of still more electropositive metals with reference to oxygen, subjecting such metal oxides or compounds thus liquefied below their normal melting-point to the action of an electrolytic current capable of dissociating them with or without the employment of electrodes capable of uniting with the electronegative constituents evolved.

My invention relates particularly to the production of aluminium alloys from metal aluminates, but is not confined thereto, as it may be applied to the reduction of many other metals and production of other alloys.

In carrying out my invention for the production of aluminium alloys I take oxides of lithium and calcium in proportion of about four of the former to one of the latter and fuse the same by any economical means, such as heat externally applied or preferably by the passage of an alternating electric current through the same, between electrodes, the said alternating current being of such character that it will not yield metal from the substances fused thereby. Then after fusion I add to the bath an aluminate of the metal an alloy of which with aluminium is desired, which readily dissolves therein, and simultaneously subject such dissolved aluminate, which has been liquefied below its normal melting-point by the action of the associated solvent substances, to the action of a current of electricity capable of electrolyzing the liquefied aluminate and yielding or liberating an aluminium alloy therefrom.

It should be noted that the solvent bath of metal oxides employed in the reduction of metals must consist of oxides of metals which have a greater affinity for oxygen than does

the metals desired to be reduced or alloys thereof produced, the principal metals having greater affinity for oxygen than aluminium being lithium, calcium, and magnesium. I prefer, however, to form the solvent bath for the reduction of aluminates of a mixture or combination of lithium and calcium oxides, as before stated, for the reason that the lithium oxide reduces the density or specific gravity of the calcium oxide, as well as its melting-point, and allows the aluminium alloy liberated within its mass by decomposition of the aluminate to readily settle to the bottom thereof, so that it can be withdrawn from time to time, as desired, without fear of loss by oxidation, which would result should the metal remain suspended within a more dense molten material for any length of time, whereby it might reach the surface through circulation and burn in the presence of the oxygen of the air and also prevents final loss of metal, which might otherwise remain mixed with the fluxes on cooling. Lithium oxide and calcium oxide may be employed *per se* as a solvent bath; but I prefer the mixture as aforesaid and for the reasons noted.

In carrying out my process for the production of aluminium alloys I prefer to employ an apparatus as illustrated in the accompanying drawings, in which—

Figure 1 is a plan or top view. Fig. 2 is a vertical section on the line R R, Fig. 1. Fig. 3 is a longitudinal vertical section on the line S S, Fig. 1. Figs. 4, 5, 6, and 7 illustrate various means of applying an alternating current to the solvent chemical bath of oxides for the purpose of melting the same.

In referring to the figures aforementioned the letter A designates a box or receptacle, preferably of iron, lined with a substance, such as carbon B, in such a manner as to form a receptacle for the substances to be reduced and solvent chemical bath therefor, in which is an electric conductor and a resistant, preferably of fusible nature, such as aluminium, and lithium, and calcium oxides in proportion of about four of the former to one of the latter and communicating with the electrodes. The material, such as the mixture of lithium and calcium oxides, as before stated, is introduced in the apparatus through the openings E, which are closed by the insulating-covers or plugs F passing in the insulating-cover X, through which passes the electrodes G and T,

which electrodes preferably consist of or contain carbon. The box or receptacle A is connected as cathode, while the electrodes G are connected as anode, when employing a direct current in an electric circuit for electrolyzing or dissociating aluminium oxid or other metal-containing oxy compound. In starting the apparatus I pass through the alternate carbon-rods or electrodes T and the carbon lining of the box A an alternating electric current of such character that it will not yield metal from the substances employed and start an arc between the said electrodes T and the inside of the receptacle of the carbon-lined box A by separating the said electrodes T slightly from contact with the carbon lining of the receptacle and then feed in lithium and calcium oxids, which quickly become fused and accumulates in the carbon-lined receptacle, communicating with the electrodes T, through which after fusion the current of electricity passes as the electrodes are separated farther and farther from the interior of the carbon-lined receptacle and through which between the electrodes the alternating current passes, producing heat enough to fuse and maintain fusion of the solvent chemical bath without decomposition. When the solvent bath has become suitably fused, I then disconnect the alternating or non-metal-yielding current from contact with the furnace-lining B and alternately connect the electrodes T, making each alternate electrode T constitute the direct terminus, communicating with the opposite poles of the alternating or non-metal-yielding current-generator in such a manner that the non-metal-yielding current will pass from and to the alternate electrodes T through the fused substance under the electrodes G, by which electrodes G a direct current is passed through the molten bath from the furnace-lining which constitutes the cathode, the alternating heating or non-metal-yielding current being passed in a direction through the fused conductor in a path disposed at an angle to the path of the direct or metal-yielding current, as indicated by the small arrows passing through the bath between the contacts T, as shown in Fig. 4. I then introduce from time to time into the molten chemical bath through the openings E by removing the insulated covers or plugs F a metal aluminate, such as copper aluminate, which almost immediately becomes liquefied by the action of the solvent bath. As the metal aluminate, such as copper aluminate, becomes liquefied by the action of the chemical solvent bath I pass through the molten bath a direct or electrolytic current of electricity between the anodes G and the carbon lining B, which constitutes the cathode. By this procedure I am enabled to maintain a fluid condition of the solvent bath at a temperature below the normal melting-point of the metal aluminate by the action 65 of an alternating current incapable of yield-

ing metal from the substance employed, while the whole of the direct current may be utilized for electrolytic purposes in dissociating or electrolyzing the metal aluminate which has been liquefied by the action of the chemical bath below its normal melting-point. The great advantage gained by such operation will be seen when the cheapness with which an alternating current may be produced, transmitted, and employed for heating purposes is compared with the more expensive direct current, which more expensive direct current may be wholly employed for the purpose of electrolytical dissociation in the liberation of the aluminium alloy without loss. 70 The aluminium alloy or other metal reduced is withdrawn from time to time, as desired, through the tap-hole K and trough L by removing the plug I, the gaseous by-products escaping through the conduits M N. 75

In Figs. 5, 6, and 7 I have illustrated another means whereby the substances are maintained in a molten condition by passing therethrough an alternating or non-metal-yielding current of electricity between the electrodes T independent of and insulated from the furnace by the insulation O. By the means here illustrated all of the vertical carbon electrodes G may be connected as anode in the circuit of the direct current, thereby admitting of a 90 larger electrolytic yield. In these figures—namely, 5, 6, and 7—similar letters of reference constitute corresponding parts with those of 1, 2, 3, and 4.

When lithium and calcium oxids are fused 100 together to form my preferable solvent bath for aluminates, as hereinbefore described, they appear to combine to form a solvent bath which dissolves the aluminate without further combination or reaction or, in other 105 words, is inert thereto. By adding copper oxid with aluminium oxid or copper aluminate to the solvent oxy-bath copper-aluminium alloys may be produced by electrolysis, or by adding aluminates of other metals or mixtures 110 of other oxides of metals to which aluminium oxid acts as acid other aluminium alloys may be produced. I can also employ instead of aluminates or compositions of aluminium oxid with other metals the oxid or oxides of 115 other metals combined with other metals—such as chromates, vanadates, stanates, tungstates, molybdates, &c.—the alloys of which are desired so long as their reduction is performed in a bath of solvent oxides of metal 120 having greater affinity for oxygen than the metal or metals the alloy of which is desired.

My invention, specifically stated, therefore, consists in exposing a molten body of metal oxides to the action of an electrolytic current 125 capable of selectively separating two or more of the metals therefrom without reducing the metal having greater affinity for oxygen, while replenishing the bath from time to time with an oxy compound of the metal or metals 130

desired, the solvent bath in which the electrolysis of the metals is performed consisting of fused oxy compounds of metals having greater affinity for oxygen than the metal or 5 metals desired.

It has nowhere in prior art been anticipated to form a bath for aluminates or compounds of metal oxide with other metals by fusing the combined oxides of metals and liquefying the 10 metal compound, the metal or alloy of which is desired, below its normal melting-point by adding it to the fused oxide bath and subjecting the metal compound thus dissolved to the action of a direct current of electricity capable of yielding or liberating the metal by 15 electrolysis, whereby the aluminate or other metal oxy compound may be reduced continuously by supplying it from time to time to the fused oxide solvent bath as increments are reduced to a metallic state as performed by my 20 process. By maintaining a relatively low voltage of the direct or electrolytic current the aluminates, &c., may be readily dissociated, liberating aluminium or other alloys without 25 deteriorating or decomposing the solvent oxide bath because of the greater affinity of the metals of the solvent bath for oxygen.

A further important and novel feature of my process is that I fuse and maintain fusion of 30 the solvent chemical bath by the action of an alternating electric current or one incapable of yielding metal passed through the same between electrodes and reduce the metal from the oxy compound contained in the fused bath 35 by the action of an electric current capable of yielding metal therefrom.

Instead of employing as a chemical solvent bath fused lithium and calcium oxides, or what may be termed "lithium calcate," or substance 40 containing the same, as herein set forth, I can employ fused lithium glucinum oxides or lithium glucinate or substance containing the same in cases where particular lightness or low specific gravity of the bath is desired, or 45 I can employ fused lithium hydrogen oxides or lithium hydrate, hydrogen being considered as a metal, or I can mix or combine any oxid or oxides or compositions thereof or employ any oxy compound of metal in a fused 50 condition as a chemical bath in which the reduction of metal is performed, so long as the said fused bath consists of an oxy compound or compounds of metal having greater affinity for oxygen under the existing conditions than 55 the metal desired, and the direct or electrolytic current is so regulated as to decompose or liberate metal or metals therefrom having less affinity for oxygen than the metal or 60 metals of the fused bath under its existing condition without departing from the spirit of my invention.

In the reduction of refractory metal oxides, such as aluminates dissolved in a molten bath of chemicals, as hereinbefore set forth, the 65 refractory metal oxy compound is dissolved

by the solvent action of the fused chemical solvent, and its liquefaction below its normal melting-point is accomplished by the direct solvent action of the chemical bath without the expenditure of either heat or electrical 70 energy to accomplish its fusion. The liquefaction of refractory metal oxide is therefore accomplished by means other than the action of an electric current.

It will be noted that the non-metal-yielding 75 current employed for fusing and maintaining the fusion of metal-containing substances employed in my process is passed through the fused substances between contacts in such a manner that its path is at an angle to the path 80 of the direct or metal-yielding current. The advantage of disposing the non-metal-yielding current employed for fusion purposes at an angle to the direct or metal-yielding current may be seen when it is understood that during 85 the employment of a direct current for fusion and electrolytic purposes should the metal-yielding current be checked for a short period the fused substances in the path thereof have a tendency to solidify and become non-conductive, thereby insulating the electrodes from 90 each other, occasioning great loss of time and energy to reestablish the flow of current between the same. Therefore by so disposing the fusing or non-metal-yielding current that 95 its path is at an angle to the path of the direct or metal-yielding current the maintenance of the fusion of the substances is assured and the difficulty experienced in the prior art is obviated.

Having now described my invention, what 100 I claim as new, and desire to secure by Letters Patent, is—

1. The process of reducing metal from substances containing the same which consists in fusing the metal-containing substance by passing 105 a non-metal-yielding current through the fused material between contacts, and liberating the metal from its compound by the action of a metal-yielding current passed therethrough in a path disposed at an angle to the 110 path of the heating or non-metal-yielding current.

2. The process of reducing aluminium from substances containing the same which consists in fusing an aluminium-containing substance 115 by passing a non-metal-yielding current through the fused material between contacts, and liberating the aluminium from its compound by the action of a metal-yielding current passed therethrough in a path disposed 120 at an angle to the path of the heating or non-metal-yielding current.

3. The process of reducing metal from substances containing the same which consists in liberating the metal by the action of a metal-yielding current while traversing a fused metal-containing substance between contacts with an alternating current at an angle to the 125 path of the metal-yielding current.

4. The process of reducing metal from sub- 130

stances containing the same which consists in liberating the metal by the action of a metal-yielding current while traversing the fused metal-containing substance between contacts  
5 with a non-metal-yielding current disposed at an angle to the path of the metal-yielding current.

In testimony whereof I affix my signature in presence of two witnesses.

HENRY SPENCER BLACKMORE.

Witnesses:

C. C. WRIGHT,  
C. M. FORREST.